

Aug. 5, 1952

P. PAYSON

2,606,113

AGE HARDENING AUSTENITIC STEEL

Filed Dec. 20, 1947

*Fig. 1.*

BAR 5173- .16C; 25.0 Ni; 20.8 Cr; 3.5 Al.  
SOLUTION TREATED - 2200°F.



*Fig. 2.*

BAR 5178-25C; 24.5 Ni; 21.3 Cr; 3.5 Al; 2.6 Mo.  
SOLUTION TREATED 2300°F.



INVENTOR.

PETER PAYSON.

BY

Wood, Cooley & Head

ATTORNEYS.

1. A heat-treatable austenitic steel having a composition by weight of 18 to 22% chromium, 8 to 12% nickel, 0.1 to 1% carbon, 0.5 to 1.5% manganese, 0.5 to 1.5% aluminum, 0.5 to 1.5% molybdenum and/or tungsten, and 0.1 to 0.5% iron, the steel being heat-treated to a temperature of 1100° F. to 1400° F. for a period of time sufficient to cause a marked increase in hardness, the steel being substantially free of martensite.

2. A heat-treatable austenitic steel having a composition by weight of 18 to 22% chromium, 8 to 12% nickel, 0.1 to 1% carbon, 0.5 to 1.5% manganese, 0.5 to 1.5% aluminum, 0.5 to 1.5% molybdenum and/or tungsten, and 0.1 to 0.5% iron, the steel being heat-treated to a temperature of 1100° F. to 1400° F. for a period of time sufficient to cause a marked increase in hardness, the steel being substantially free of martensite, the steel having a balance of iron.

# UNITED STATES PATENT OFFICE

2,606,113

## AGE HARDENING AUSTENITIC STEEL

Peter Payson, New York, N. Y., assignor to Crucible Steel Company of America, New York, N. Y., a corporation of New Jersey

Application December 20, 1947, Serial No. 792,929

2 Claims. (Cl. 75—124)

1

This invention pertains to hardenable, corrosion and heat-resisting austenitic steels, and more particularly to a steel of this character which can be forged and rolled, and which, as annealed or solution-treated, is quite soft so that it can be cold-formed readily, or machined, and which can subsequently be hardened to Rockwell "C" 30 or 40 or higher, depending upon the analysis, by heat treatment at relatively low temperatures.

The essentially straight chromium hardenable stainless steels, such as A. I. S. I. types 410, 420 and 440, i. e., those containing about 12 to 18% chromium with carbon about 0.1 to 1%, or the chromium-nickel steel type 431 containing about 16% chromium, 2% nickel and 0.1 to 0.2% carbon, have to be treated to temperatures in excess of 1700° F. as a necessary step for hardening. This generally entails serious oxidation or discoloration of the surface, requiring final cleaning and polishing to confer the desired metallic luster and corrosion-resistance to articles made therefrom. These steels harden by martensite formation, and the hardening thereof without discoloration must be effected in special atmosphere furnaces, which are ordinarily not readily available. Furthermore, even the best of these steels, when properly heat treated and polished, have limited resistance to corrosion, as indicated for example in the 20% sodium chloride spray test.

The austenitic stainless steels of which A. I. S. I. types 302, 310 and 316 are examples, i. e., 18-8, 25-20 and 18-12 with molybdenum, respectively, when in the annealed or solution-treated condition, are easy to cold-work and machine, but they can be hardened only by severe cold-rolling or drawing operations. Articles of appreciable strength and wear-resistance can therefore be made from these steels only in simple sections which can be cold-rolled or cold-drawn. These steels, which are highly resistant to corrosion as well as to oxidation at high temperatures, are therefore limited in their usefulness for articles of high strength.

Steels are known, as for example those de-

scribed in French Patent 743,179, which are stainless and hardenable to an appreciable degree by a heat treatment causing a phase change from unstable austenite to martensite. But such steels have the disadvantage that they are not readily workable by cold-forming or machining since, being borderline alloys, they tend to harden by martensite formation while they are being worked. Other stainless steels are known, as for example those described in U. S. Patent 2,381,416, which harden appreciably by aging of stress-laden ferrite. Such steels also have the disadvantage mentioned above of not being readily workable because they are fairly hard, about Rockwell "C" 23, prior to the aging treatment. Finally, there are known stainless steels of sufficient alloy content to be substantially austenitic, and which may be hardened somewhat by aging without any change from austenite to the ferritic phase. However, the known steels of this type do not harden sufficiently to be of appreciable use in industry.

Now I have discovered, in accordance with the present invention, that there are certain steel compositions which, by virtue of the balance of nickel, chromium and aluminum, and in some analyses also molybdenum, present in the steel, have a soft, ductile and substantially austenitic structure, as annealed or solution-treated, and which undergo a marked increase in hardness from about Rockwell "B" 85 or softer, to Rockwell "C" 30 or 40 or harder, by an aging treatment at about 1100° to 1400° F., without the formation of martensite or any other ferritic product from the austenite.

The steels which I have discovered to possess these properties are those within the following range of analysis, constituting the broad range of analysis of my invention, viz:

|    |                            |                    |
|----|----------------------------|--------------------|
| 40 | Carbon                     | Up to about 0.4%   |
|    | Manganese + nickel         | About 20 to 30%    |
|    | Chromium                   | About 15 to 25%    |
|    | Aluminum                   | About 2.5 to 4.5%  |
| 45 | Molybdenum and/or tungsten | Up to about 5%     |
|    | Balance                    | Substantially iron |

It will be understood that by specifying the balance as "substantially iron" is meant iron containing the usual amounts of silicon and residual elements ordinarily found in high quality steel. The preferred composition for one of the lower cost varieties of this steel is:

|           |                    |
|-----------|--------------------|
| Carbon    | About .10 to .25%  |
| Manganese | About 1.0 to 2.0%  |
| Silicon   | About .20 to .50%  |
| Nickel    | About 22 to 24%    |
| Chromium  | About 20 to 22%    |
| Aluminum  | About 3 to 4%      |
| Balance   | Substantially iron |

And for a steel which attains a somewhat higher hardness, and which has better corrosion resistance, and better strength at elevated temperatures, the preferred composition is:

|            |                    |
|------------|--------------------|
| Carbon     | About .10 to .25%  |
| Manganese  | About 1 to 2%      |
| Silicon    | About .20 to .50%  |
| Nickel     | About 24 to 26%    |
| Chromium   | About 19 to 21%    |
| Aluminum   | About 3 to 4%      |
| Molybdenum | About 2 to 4%      |
| Balance    | Substantially iron |

These steels can be hardened respectively from Rockwell "B" 83 as solution-treated at 2200° F., to Rockwell "C" 40 as aged at 1300° F. for 8 hours; and from Rockwell "B" 87 as solution-treated at 2300° F., to Rockwell "C" 43 as aged at 1400° F. for 8 hours. The maximum hardnesses attainable are even higher for longer aging times and somewhat lower aging temperatures. That this hardening is strictly age hardening without phase change is substantiated by the facts that the changes in hardness with time and temperature of aging as shown in Figures 1 and 2 of the accompanying drawing, follow the classic pattern for age hardening alloys discussed by E. S. Davenport and E. C. Bain in the article "The Aging of Steel" in Transactions of the American Society for Metals, volume 23, 1935, pages 1047 to 1096; and that the steel remain substantially non-magnetic after the hardening is completed.

The "balance" in relative proportions of the various elements aforesaid in the steel of the invention, is quite important for the production of the desired forgeable, corrosion and heat resisting properties, including a soft and substantially austenitic structure as solution treated, but which can be hardened appreciably by aging at a relatively low temperature. As the carbon is increased, the forgeability decreases and the aforesaid high nickel, chromium, aluminum, molybdenum analyses become practically non-forgeable when the carbon is over about 0.40%. Forgeability is also rapidly impaired as the aluminum content exceeds about 4.5% and the molybdenum content exceeds about 5.0%. When steels of the general type aforesaid contain appreciable amounts of aluminum, they are strongly magnetic, that is, not substantially austenitic as is desired in steels that are easy to cold-work, if the nickel plus manganese content is below that of the chromium content. For example, the steels shown in Table 1 were definitely magnetic as solution treated at 2100° F.

TABLE 1.—NON-AUSTENITIC Ni—Cr—Al STEELS

|    | Bar  | C   | Mn   | Si  | Ni    | Cr    | Al   |
|----|------|-----|------|-----|-------|-------|------|
| 10 | 8777 | .10 | 1.43 | .30 | 14.66 | 18.36 | 3.10 |
|    | 8772 | .08 | 1.41 | .39 | 17.55 | 18.56 | 3.20 |
|    | 8116 | .15 | 1.33 | .44 | 14.19 | 20.24 | 3.70 |
|    | 5117 | .14 | 1.37 | .49 | 18.86 | 20.52 | 3.75 |
|    | 5118 | .15 | 1.41 | .55 | 20.45 | 20.25 | 3.57 |
|    | 5119 | .13 | 1.46 | .50 | 14.53 | 22.52 | 3.60 |
|    | 5120 | .14 | 1.48 | .54 | 17.04 | 22.60 | 3.53 |

On the other hand, when the nickel plus manganese content is above that of the chromium content, the steels with high aluminum content are substantially non-magnetic or austenitic. Examples of such steels are given in Tables 2 to 10.

In the substantially austenitic nickel-chromium-aluminum steels, there is a minimum amount of aluminum required to confer appreciable hardening of the steel by aging, as shown in Table 2.

TABLE 2.—SUBSTANTIALLY AUSTENITIC Ni—Cr—Al STEELS

*Effect of Al content on hardening by aging*

[Samples solution treated at 2100° F. and aged at 1300° F. for 16 hours]

|    | Bar  | Percent C | Percent Mn | Percent Si | Percent Ni | Percent Cr | Percent Al | Rockwell Hardness |
|----|------|-----------|------------|------------|------------|------------|------------|-------------------|
| 35 | 8778 | .11       | 1.48       | .42        | 23.47      | 18.48      | 1.09       | B 84              |
|    | 8779 | .11       | 1.47       | .29        | 23.47      | 18.67      | 1.98       | C 7               |
|    | 8837 | .11       | 1.51       | .36        | 22.73      | 18.30      | 2.56       | C 23              |
|    | 8613 | .10       | 1.36       | .39        | 23.17      | 19.00      | 3.10       | C 33              |
|    | 8836 | .12       | 1.45       | .31        | 25.83      | 18.06      | 4.36       | C 38              |
| 40 |      |           |            |            |            |            |            |                   |

Also in the substantially austenitic steels containing aluminum, the degree of age hardening is dependent on the chromium content as is shown in Table 3.

TABLE 3.—SUBSTANTIALLY AUSTENITIC Ni—Cr—Al STEELS

*Effect of Cr content on hardening by aging*

[Samples solution treated at 2100° F. and aged at 1300° F. for 16 hours]

|    | Bar  | Percent C | Percent Mn | Percent Si | Percent Ni | Percent Cr | Percent Al | Percent Mo | Rockwell Hardness |
|----|------|-----------|------------|------------|------------|------------|------------|------------|-------------------|
| 55 | 8838 | .10       | 1.46       | .39        | 23.19      | 15.57      | 2.92       | -----      | C 24              |
|    | 8613 | .10       | 1.36       | .30        | 23.17      | 19.00      | 3.10       | -----      | C 33              |
|    | 8839 | .10       | 1.50       | .39        | 22.73      | 21.05      | 3.09       | -----      | C 38              |
|    | 5230 | .17       | 1.35       | .49        | 22.79      | 21.03      | 3.44       | -----      | C 38              |
|    | 5007 | .08       | 1.39       | .47        | 24.29      | 16.37      | 3.14       | -----      | C 24              |
|    | 5008 | .10       | 1.49       | .43        | 24.06      | 19.21      | 3.17       | -----      | C 24              |
|    | 5009 | .10       | 1.49       | .42        | 23.66      | 19.78      | 3.35       | -----      | C 31              |
|    | 5010 | .12       | 1.53       | .45        | 24.52      | 22.07      | 3.30       | -----      | C 34              |
|    | 5016 | .11       | 1.52       | .36        | 25.61      | 16.33      | 3.76       | 2.96       | C 36              |
|    | 5012 | .09       | 1.46       | .45        | 25.30      | 18.39      | 3.65       | 2.83       | C 32              |
|    | 5017 | .11       | 1.63       | .38        | 25.37      | 20.16      | 3.74       | 2.96       | C 37              |
| 65 |      |           |            |            |            |            |            |            | C 40              |

These data show that attainable hardness by aging increases with increasing chromium. However, it has been found that when chromium is over about 23.0%, the forgeability of the steel rapidly deteriorates.

An addition of molybdenum (or tungsten) to the substantially austenitic nickel-chromium-aluminum steels increases the attainable hardness by aging as shown in Table 4.

TABLE 4.—SUBSTANTIALLY AUSTENITIC Ni—Cr—Al—Mo STEELS

*Effect of Mo content on hardening by aging*

[Samples solution treated at 2300° F. and aged at 1400° F. for 16 hours]

| Bar  | Percent C | Percent Mn | Percent Si | Percent Ni | Percent Cr | Percent Al | Percent Mo | Rockwell Hardness | 10   | Bar | Percent C | Percent Mn | Percent Si | Percent Ni | Percent Cr | Percent Al | Percent Mo | Rockwell C Hardness |
|------|-----------|------------|------------|------------|------------|------------|------------|-------------------|------|-----|-----------|------------|------------|------------|------------|------------|------------|---------------------|
| 8846 | .11       | 1.45       | .32        | 25.31      | 18.49      | 2.63       | —          | C 23              | 5056 | .09 | 1.42      | .38        | 24.84      | 20.00      | 3.61       | 2.77       | 40         |                     |
| 8847 | .11       | 1.41       | .35        | 25.88      | 19.12      | 2.76       | 2.65       | C 34              | 5177 | .20 | 1.35      | .52        | 24.72      | 20.77      | 3.14       | 2.51       | 37         |                     |
| 8848 | .12       | 1.41       | .41        | 25.48      | 18.46      | 2.65       | 6.54       | C 42              | 5178 | .25 | 1.37      | .50        | 24.50      | 20.95      | 3.58       | 2.60       | 43         |                     |
| 8849 | .14       | 1.44       | .34        | 24.97      | 18.36      | 2.79       | 8.53       | C 47              | 5179 | .33 | 1.37      | .53        | 24.53      | 21.25      | 3.49       | 2.58       | 41         |                     |
| 8854 | .13       | 1.50       | .35        | 28.50      | 19.98      | 3.36       | —          | C 27              | 15   | —   | —         | —          | —          | —          | —          | —          | —          |                     |
| 8855 | .15       | 1.46       | .35        | 28.61      | 18.56      | 3.01       | 3.10       | C 32              | —    | —   | —         | —          | —          | —          | —          | —          | —          |                     |
| 8856 | .14       | 1.46       | .41        | 28.73      | 18.63      | 2.80       | 6.59       | C 42              | —    | —   | —         | —          | —          | —          | —          | —          | —          |                     |
| 8857 | .14       | 1.47       | .36        | 29.18      | 19.32      | 2.96       | 8.61       | C 48              | —    | —   | —         | —          | —          | —          | —          | —          | —          |                     |

It is shown above that the attainable hardness by aging increases with increasing molybdenum. However, it has been found that the forgeability decreases also with increasing molybdenum, and steels with more than about 5.0% molybdenum can be forged only with difficulty, and those with molybdenum around 10% can be forged hardly at all.

The effect of carbon on the attainable hardness by aging is practically negligible as shown in the following Tables 5 and 6.

TABLE 5.—SUBSTANTIALLY AUSTENITIC Ni—Cr—Al STEELS

*Effect of C content on hardening by aging*

[Samples solution treated at 2200° F. and aged at 1300° F. for 16 hours]

| Bar  | Percent C | Percent Mn | Percent Si | Percent Ni | Percent Cr | Percent Al | Rockwell C Hardness |
|------|-----------|------------|------------|------------|------------|------------|---------------------|
| 5169 | .10       | 1.23       | .50        | 24.70      | 20.64      | 3.13       | 34                  |
| 5170 | .17       | 1.35       | .55        | 24.64      | 20.49      | 2.96       | 36                  |
| 5171 | .23       | 1.36       | .56        | 24.23      | 21.37      | 3.01       | 38                  |
| 5172 | .09       | 1.28       | .54        | 24.60      | 20.70      | 3.41       | 40                  |
| 5173 | .16       | 1.34       | .55        | 24.97      | 20.84      | 3.52       | 42                  |
| 5174 | .24       | 1.26       | .53        | 25.37      | 20.11      | 3.35       | 39                  |
| 5175 | .32       | 1.32       | .58        | 24.98      | 20.81      | 3.67       | 40                  |
| 5176 | .39       | 1.33       | .60        | 24.58      | 21.18      | 3.32       | 39                  |

TABLE 6.—SUBSTANTIALLY AUSTENITIC Ni—Cr—Al—Mo STEELS

*Effect of C content on hardening by aging*

[Samples solution treated at 2300° F. and aged at 1400° F. for 16 hours]

| Bar  | Percent C | Percent Mn | Percent Si | Percent Ni | Percent Cr | Percent Al | Percent Mo | Rockwell C Hardness |     |     |     |     |     |     |     |
|------|-----------|------------|------------|------------|------------|------------|------------|---------------------|-----|-----|-----|-----|-----|-----|-----|
| 5056 | .09       | 24.8       | 20.0       | 3.6        | 2.8        | B92        | B90        | B83                 | B80 | B80 | C37 | C40 | C41 | C42 | C43 |
| 5057 | .09       | 24.9       | 20.5       | 3.4        | 3.6        | B96        | B91        | B89                 | B87 | B87 | C39 | C43 | C43 | C44 | C45 |
| 5098 | .09       | 24.9       | 22.7       | 3.2        | 2.8        | B95        | B90        | B88                 | B88 | B88 | C40 | C42 | C42 | C42 | C42 |
| 5058 | .09       | 27.4       | 20.9       | 3.2        | 2.8        | B80        | B79        | B78                 | B75 | B72 | C37 | C38 | C39 | C39 | C41 |
| 5059 | .09       | 28.0       | 20.1       | 3.3        | 3.7        | B83        | B80        | B79                 | B77 | B74 | C39 | C40 | C41 | C41 | C43 |
| 5060 | .10       | 28.1       | 23.2       | 3.2        | 2.8        | C21        | B92        | B88                 | B83 | B83 | C40 | C41 | C42 | C43 | C43 |

The forgeability of these steels is, however, affected by carbon content, particularly in the steels containing molybdenum, and is progressively worse with increasing carbon. When the carbon is over about 0.40%, the steel is hardly forgeable.

Finally, the effect of increasing nickel above about 30.0% is generally to decrease the hardness attainable by aging in these steels, as shown in the following Table 7.

TABLE 7.—SUBSTANTIALLY AUSTENITIC Ni—Cr—Al STEELS

*Effect of Ni content on hardening by aging*

[Samples solution treated at 2100° F. and aged at 1300° F. for 16 hours]

| Bar  | Percent C | Percent Mn | Percent Si | Percent Ni | Percent Cr | Percent Al | Rockwell C Hardness |
|------|-----------|------------|------------|------------|------------|------------|---------------------|
| 8773 | .10       | 1.47       | .37        | 20.01      | 18.60      | 3.16       | 30                  |
| 8774 | .09       | 1.45       | .34        | 25.58      | 18.84      | 3.11       | 28                  |
| 8775 | .11       | 1.50       | .35        | 29.04      | 19.06      | 3.04       | 29                  |
| 8776 | .10       | 1.51       | .31        | 31.72      | 18.68      | 3.09       | 22                  |

The temperature for annealing or solution treating these substantially austenitic nickel-chromium-aluminum-molybdenum steels may be between about 1900° and 2400° F. but preferably between 2100° and 2300° F., the steels containing molybdenum requiring the higher temperatures. The effect of solution temperature on the hardness as annealed and after aging is shown in the following Table 8.

TABLE 8.—SUBSTANTIALLY AUSTENITIC Ni—Cr—Al STEELS

*Effect of solution treatment on hardness before and after aging*

[Samples solution treated at 1900° to 2300° F. and aged for 18 hours at 1350° F.]

| Bar  | Percent |      |      |     |     | Rockwell Hardness |      |      |      |      |      |      |      |      |      |  |  |
|------|---------|------|------|-----|-----|-------------------|------|------|------|------|------|------|------|------|------|--|--|
|      | C       | Ni   | Cr   | Al  | Mo  | 1900              | 2000 | 2100 | 2200 | 2300 | 1900 | 2000 | 2100 | 2200 | 2300 |  |  |
| 5056 | .09     | 24.8 | 20.0 | 3.6 | 2.8 | B92               | B90  | B83  | B80  | B80  | C37  | C40  | C41  | C42  | C43  |  |  |
| 5057 | .09     | 24.9 | 20.5 | 3.4 | 3.6 | B96               | B91  | B89  | B87  | B87  | C39  | C43  | C43  | C44  | C45  |  |  |
| 5098 | .09     | 24.9 | 22.7 | 3.2 | 2.8 | B95               | B90  | B88  | B88  | B88  | C40  | C42  | C42  | C42  | C42  |  |  |
| 5058 | .09     | 27.4 | 20.9 | 3.2 | 2.8 | B80               | B79  | B78  | B75  | B72  | C37  | C38  | C39  | C39  | C41  |  |  |
| 5059 | .09     | 28.0 | 20.1 | 3.3 | 3.7 | B83               | B80  | B79  | B77  | B74  | C39  | C40  | C41  | C41  | C43  |  |  |
| 5060 | .10     | 28.1 | 23.2 | 3.2 | 2.8 | C21               | B92  | B88  | B83  | B83  | C40  | C41  | C42  | C43  | C43  |  |  |

The best aging treatments for these steels is between about 1200° and 1500° F., the molybdenum steels requiring a somewhat higher temperature than the steels without molybdenum, as shown in the following Table 9.

2 to 4% of metal of the group molybdenum and tungsten; about 0.1 to 0.25% carbon; and the balance substantially all iron.

2. A forgeable and machinable, age hardening, heat and corrosion-resisting alloy steel, charac-

TABLE 9.—SUBSTANTIALLY AUSTENITIC  
Ni—Cr—Al—Mo STEELS

*Effect of solution and aging treatments on attainable hardness*

[Rockwell hardness; "C" except as indicated]

| Bar      | Aging<br>Time<br>Hours | Sol. Tr. at 2100° F;<br>aged at— |     |     |   | Sol. Tr. at 2200° F;<br>aged at— |     |     |   | Sol. Tr. at 2300° F;<br>aged at— |     |     |   |
|----------|------------------------|----------------------------------|-----|-----|---|----------------------------------|-----|-----|---|----------------------------------|-----|-----|---|
|          |                        | 1200° 1300° 1400° 1500°          |     |     |   | 1200° 1300° 1400° 1500°          |     |     |   | 1200° 1300° 1400° 1500°          |     |     |   |
|          |                        | B81                              | B81 | B81 | — | B77                              | B77 | B77 | — | B74                              | B74 | B74 | — |
| Bar 5172 | 0                      | B81                              | B81 | B81 | — | B77                              | B77 | B77 | — | B74                              | B74 | B74 | — |
| C .09    | 4                      | 19                               | 33  | 35  | — | 15                               | 37  | 36  | — | 13                               | 34  | 37  | — |
| Ni 24.6  | 16                     | 29                               | 38  | 32  | — | 28                               | 39  | 33  | — | 27                               | 39  | 33  | — |
| Cr 20.7  | 48                     | 36                               | 36  | 32  | — | 38                               | 38  | 32  | — | 39                               | 37  | 33  | — |
| Al 3.4   | 208                    | 41                               | 33  | 29  | — | 40                               | 34  | 29  | — | 40                               | 34  | 30  | — |
| Bar 5173 | 0                      | 7                                | 7   | 7   | — | 3                                | 3   | 3   | — | B78                              | B78 | B78 | — |
| C .16    | 4                      | 27                               | 35  | 34  | — | 25                               | 38  | 37  | — | 18                               | 39  | 38  | — |
| Ni 25.0  | 16                     | 32                               | 38  | 32  | — | 33                               | 39  | 34  | — | 34                               | 40  | 35  | — |
| Cr 20.8  | 48                     | 37                               | 35  | 32  | — | 40                               | 38  | 34  | — | 42                               | 39  | 35  | — |
| Al 3.5   | 208                    | 41                               | 32  | 29  | — | 41                               | 34  | 31  | — | 41                               | 36  | 31  | — |
| Bar 5178 | 0                      | 12                               | 12  | 12  | — | 10                               | 10  | 10  | — | 8                                | 8   | 8   | — |
| C 0.25   | 4                      | 32                               | 40  | 39  | — | 28                               | 41  | 40  | — | 27                               | 43  | 41  | — |
| Ni 24.5  | 16                     | 35                               | 42  | 40  | — | 34                               | 35  | 43  | — | 38                               | 44  | 42  | — |
| Cr 21.0  | 48                     | 39                               | 43  | 40  | — | 34                               | 41  | 43  | — | 36                               | 45  | 42  | — |
| Al 3.6   | 208                    | 43                               | 41  | 37  | — | 44                               | 42  | 38  | — | 46                               | 44  | 40  | — |
| Mo 2.6   | —                      | —                                | —   | —   | — | —                                | —   | —   | — | —                                | —   | —   | — |

Both Tables 8 and 9 emphasize the truly remarkable degree to which these properly balanced steels harden by aging.

That these steels as aged are really high strength corrosion resistant materials are evidenced by the mechanical properties data in Table 10, and by the fact that as age hardened, these steels are equivalent to the well known 18-8 Stainless Steel, as annealed in corrosion resistance to a spray made up of 20% sodium chloride.

30 terized in being ductile, substantially austenitic and having a hardness below about "B" 90 Rockwell, as solution treated at about 1900 to 2400° F., and in being hardenable in excess of "C" 30 Rockwell on subsequent aging at about 1100 to 1500° F., said steel containing: about 24 to 26% nickel; about 1 to 2% manganese; about 19 to 21% chromium; about 3 to 4% aluminum; about 2 to 4% molybdenum; about 0.1 to 0.25% carbon; and the balance substantially all iron.

PETER PAYSON.

40

TABLE 10.—SUBSTANTIALLY AUSTENITIC  
Ni—Cr—Al STEELS

*Mechanical properties of aged steels*

[Tested as standard .505 tensile pieces and V-notch Izod pieces]

| Bar  | Percent |      |      |     | Treatment                         | Rock.<br>C | T. S.<br>p. s. i. | 0.2% YS<br>p. s. i. | EI in 2"<br>percent | R. A.<br>percent | Izod<br>ft. lbs. |
|------|---------|------|------|-----|-----------------------------------|------------|-------------------|---------------------|---------------------|------------------|------------------|
|      | C       | Ni   | Cr   | Al  |                                   |            |                   |                     |                     |                  |                  |
| 5172 | .09     | 24.6 | 20.7 | 3.4 | {2100F, water.<br>{1300F, 16 hrs. | 37         | 170,000           | 115,000             | 13.6                | 24.4             | 11               |
| 5173 | .16     | 25.0 | 20.8 | 3.5 | {2100F, water.<br>{1300F, 16 hrs. | 38         | 169,000           | 112,000             | 15.0                | 23.4             | 9                |
| 5727 | .17     | 22.8 | 21.0 | 3.4 | {1400F, 16 hrs.<br>{2200F, water. | 35         | 160,000           | 107,000             | 12.5                | 26.5             | 15               |
| 5727 | .17     | 22.8 | 21.0 | 3.4 | {2300F, water.<br>{1300F, 16 hrs. | 39         | 175,000           | 123,000             | 9.9                 | 13.0             | 11               |

As shown by the test results above presented, the steel of the invention will ordinarily contain about 20 to 30% nickel, together with about 0.5 to 5% manganese, the other constituents being as above set forth.

60

#### REFERENCES CITED

The following references are of record in the file of this patent:

#### UNITED STATES PATENTS

| 65 | Number    | Name         | Date          |
|----|-----------|--------------|---------------|
|    | 1,941,648 | Armstrong    | Jan. 2, 1934  |
|    | 2,048,167 | Pilling      | July 21, 1936 |
|    | 2,200,208 | Parsons      | May 7, 1940   |
|    | 2,381,416 | Wyche et al. | Aug. 7, 1945  |

#### FOREIGN PATENTS

| Number  | Country       | Date          |
|---------|---------------|---------------|
| 136,661 | Austria       | Oct. 15, 1933 |
| 743,179 | France        | Mar. 25, 1933 |
| 371,334 | Great Britain | Apr. 13, 1932 |

1 claim:

1. A forgeable and machinable, age hardening, heat and corrosion-resisting alloy steel, characterized in being ductile, substantially austenitic and having a hardness below about "B" 90 Rockwell, as solution treated at about 1900 to 2400° F., and in being hardenable in excess of "C" 30 Rockwell on subsequent aging at about 1100 to 1500° F., said steel containing: about 24 to 26% nickel; about 1 to 2% manganese; about 19 to 21% chromium; about 3 to 4% aluminum; about 2 to 4% molybdenum; about 0.1 to 0.25% carbon; and the balance substantially all iron.

70

2100° F., said steel containing: about 24 to 26% nickel; about 1 to 2% manganese; about 19 to 21% chromium; about 3 to 4% aluminum; about 2 to 4% molybdenum; about 0.1 to 0.25% carbon; and the balance substantially all iron.